# EUROPEAN PATENT SPECIFICATION

(11) **EP 2 481 501 B1**
(45) Date of publication and mention of the grant of the patent: **29.05.2019**
(21) Application number: 11188105.8
(22) Date of filing: 07.11.2011
(51) Int. Cl.: B22F 1/00, B22F 9/22

(54) **Synthesis method of graphitic shell-alloy core heterostructure nanowires and longitudinal metal oxide heterostructure nanowires, and reversible synthesis method between nanowires thereof**
Syntheseverfahren von Nanodrähten mit Graphithüllenlegierungskernheterostruktur und Nanodrähten mit länglicher Metalloxidheterostruktur und umkehrbares Syntheseverfahren zwischen Nanodrähten daraus
Procédé de synthèse de nano-fils d'hétérostructure de coeur d'alliage d'enveloppe graphitique et de nano-fils d'hétérostructure d'oxyde métallique longitudinal et procédé de synthèse réversible entre les nano-fils correspondant

(30) Priority: 08.11.2010 KR 20100110445; 08.11.2010 KR 20100110446
(43) Date of publication of application: 01.08.2012
(73) Proprietor: Korea Institute of Energy Research, Daejon 305-343 (KR)
(72) Inventor: Jeong, Nam Jo, 305-308 Daejeon (KR); Yeo, Jeong Gu, 301-152 Daejeon (KR); Kim, Dong Kook, 305-755 Daejeon (KR)
(74) Representative: Caspary, Karsten

(56) References cited:
- WO-A2-2010/120964
- LUBOS JANKOVIC ET AL: "Carbon Nanotubes Encapsulating Superconducting Single-Crystalline Tin Nanowires", NANO LETTERS, vol. 6, no. 6, 1 June 2006 (2006-06-01), pages 1131-1135, XP055370844, US ISSN: 1530-6984, DOI: 10.1021/nl0602387
- ANDREI KOLMAKOV ET AL: "Topotactic Thermal Oxidation of Sn Nanowires: Intermediate Suboxides and Core-Shell Metastable Structures", NANO LETTERS, vol. 3, no. 8, 1 August 2003 (2003-08-01), pages 1125-1129, XP055370853, US ISSN: 1530-6984, DOI: 10.1021/nl034321v
- CHEN S H ET AL: "Fabrication of bismuth oxide-tin oxide nanowires by direct thermal oxidation of Bi-Sn eutectic nanowires", MATERIALS LETTERS, ELSEVIER, AMSTERDAM, NL, vol. 64, no. 22, 19 August 2010 (2010-08-19), pages 2502-2504, XP027290696, ISSN: 0167-577X [retrieved on 2010-08-19]
- COMINI E ET AL: "Metal oxide nanowires: Preparation and application in gas sensing", JOURNAL OF MOLECULAR CATALYSIS A: CHEMICAL, ELSEVIER, AMSTERDAM, NL, vol. 305, no. 1-2, 15 June 2009 (2009-06-15), pages 170-177, XP026159737, ISSN: 1381-1169, DOI: 10.1016/J.MOLCATA.2009.01.009 [retrieved on 2009-01-19]

## Description

### BACKGROUND

### (a) Technical Field

The present invention relates to a method for synthesizing heterostructure nanowires that at least two kinds of substances are formed in the lateral and longitudinal directions.

In more particular, the present invention is to provide an improved method that can synthesize the heterostructure nanowires formed in lateral and longitudinal directions.

In addition, the present invention provides a synthesis method in which a reversible change can be made between a lateral heterostructure and a longitudinal heterostructure.

### (b) Background Art

Carbon nanotubes have very superior properties in the various fields of physics, machinery, chemistry and electricity and the like and can achieve very enhanced properties by combining intermetallics or alloys with CNTs.

Encapsulation of materials sensitive to environmental factors (chemical reaction, oxidation, and mechanical vulnerability) in CNT can lead the formation of new materials with more stabilized and enhanced properties, and thus heterostructure nanowires may be applied to various fields.

Heterostructure nanowires which are one-dimension nanostructure involving CNTs are typically synthesized by vapor-liquid-solid mechanism. A heterostructure nanowire is grown by absorbing and diffusing sources for nanowire growth at high temperature and therefore CNTs is formed in shell type while nanowire is grown. It is advantageous that such a synthesis method makes the heterostructure to be uniform and the control of constituent components to be easy. But it is undesirable in that this method enables the process to be complex and mass production difficult.

Another formation method of core-shell heterostructure may be accomplished by opening chemically both ends of as-synthesized CNT and then pouring new core materials into inner portion of the CNT thereof through capillary action. However, such a method provides undesirable economic efficiency and has a complex process.

A longitudinal heterostructure nanowire which is another type of heteronanowires is synthesized by a vapor-liquid-solid mechanism. In synthesis method, nano-sized catalyst particles are used, which play a role in absorbing and diffusing sources for nanowire growth.

An important feature of this synthesis method is that catalyst forms longitudinal heterostructure nanowires using gases supplied alternatively.

The above-mentioned synthesis method has advantages in that a heterostructure is uniform and control of constituent components is easy, whereas this invention has disadvantages in that process is complex and a metal should be treated above the melting point because the necessary source should be provided as gaseous phase to synthesize the heterostructure nanowires for metal, preferably, metal oxide thereby causing the problems that the energy consumption increase and a mass production is not easy in view of a characteristics of the process Jankovic et al in "Carbon Nanotubes Encapsulating Superconducting Single-Crystalline Tin Nanowires", Nano Letters, vol. 6, no. 6, pages 1131-1135, discloses a synthesis method of lateral heterostructure nanowires containing a tin core and graphitic shell.

Kolmakov et al, in "Topotactic Thermal Oxidation of Sn Nanowires: Intermediate Suboxides and Core-Shell Metastable Structures", Nano Letters, vol. 3, no. 8, pages 1125-1129 and Chen et al, in "Fabrication of bismuth oxide-tin oxide nanowires by direct thermal oxidation of Bi-Sn eutectic nanowires", Materials Letters, vol. 64, no. 22, pages 2502-2504 disclose that metal nanowires can be converted to the corresponding oxides by increasing the temperature under an oxide atmosphere.

### SUMMARY OF THE DISCLOSURE

To resolve the above noted problems, the object of the present invention is to provide a method that lateral heterostructure nanowires having graphitic shell and alloy core can be synthesized using a simple chemical vapor deposition (CVD).

In addition, the object of the present invention is to provide a method that the lateral heterotructure nanowire is oxidized to remove a graphitic shell and an alloy remained in the inner portion thereof is oxidized and separated to synthesize a longitudinal hetero nanowire.

Furthermore, the object of the present invention is to provide a reversible synthetic method that said lateral heterostructure nanowires and said longitudinal heterstructure nanowires can be converted each other.

### [Means to resolve the problem]

The present invention to achieve the above noted object provides a synthesis method of lateral heterostructure nanowires containing alloy core and graphitic shell, according to claim 1.

In addition, the present invention to achieve the above noted object provides a synthesis method of longitudinal metal oxide heterostructure nanowire, according to claim 2.

Furthermore, the present invention to achieve the above noted object provides a reversible synthesis method between graphitic shell-alloy core heterostructure nanowires and longitudinal metal oxide heterostructure nanowires, according to claim 3.

The metal oxide mixture is the mixture of indium oxide and tin oxide and is 6:1∼1:6 based on weight rate, hydrocarbon gas flowing into said reactor is one and two more mixture selected from acetylene, ethylene and methane, and the amount of hydrocarbon flowing into said reactor is preferably in the range of 2∼10 vol%.

In addition, a hydrogen gas may be flowed to assist the reaction of metal oxide mixture with hydrocarbon, and the inflow amount of said hydrogen is preferably less than 5 vol% based on a carrier gas. Furthermore, the reaction temperature of said metal oxide mixture and hydrocarbon is controlled in the range of 550∼850°C and the reaction time is preferably within 2 hours.

Moreover, the oxidation processing temperature of said graphitic shell-alloy core heterostructure nanowires is controlled in the range of 350∼650 °C. The oxidation processing time of said graphitic shell-alloy core heterostructure nanowires is preferably in the range of 1minute ∼ 6 hours, and the temperature rise for oxidation process of said graphitic shell-alloy core heterostructure nanowires is preferably made in the range of 1∼10°C/min

Furthermore, said metal oxide mixture may a mixture of bismuth oxide and tin oxide and said alloy may intermetallics .

On the other hand, graphitic shell-alloy core heterostructure nanowires synthesized using said method have superconducting critical temperature (Tc) at 4.8∼6.0 K, the outer diameter is in 50∼150 nm. the thickness of graphitic shell is 1∼20 nm, the length thereof is formed at 100nm∼10*µ*m and the inner portion of graphitic shell of the heterostructure nanowire is filled with intermetallic core more than 90%.

In addition, the longitudinal metal oxide heterostructure nanowires synthesized using said method can be of a shape that indium/tin oxide (ITO) containing tin of 0.01-10% relative to indium oxide and tin oxide is formed alternatively longitudinally, and the average diameter thereof is formed at 50∼150 nm, the length is formed at 100nm∼10*µ*m.

### BRIEF DESCRIPTION OF THE DRAWINGS

Fig. 1 is a flowchart showing the synthesis method of graphitic shell-alloy core heterostructure nanowires and longitudinal metal oxide heterostructure nanowires and the reversible synthesis method thereof.
Fig.2 shows XRD graph for lateral heterostructure nanowires having indium/tin intermetallic core and graphitic shell in accordance with the present application.
Fig.3 shows SEM image according to the synthesis temperature of lateral heterostructure nanowires having indium/tin intermetallic core and graphitic shell in accordance with the present application.
Fig.4 shows SEM image according to synthesis time of lateral heterostructure nanowires having indium/tin intermetallic core and graphitic shell in accordance with the present application.
Fig.5 shows TEM image according to the synthesis time of lateral heterostructure nanowires having indium/tin intermetallic core and graphitic shell in accordance with the present application.
Fig.6 shows the element analysis of heterostructure nanowires having indium/tin intermetallic core and graphitic shell in accordance with the present application.
Fig 7 shows XRD graph for longitudinal ITO-tin oxide heterostructure nanowires
Fig. 8 shows SEM image for longitudinal ITO-tin oxide heterostructure nanowires obtained using oxidation process of lateral heterostructure nanowires having indium/tin core and graphitic shell in accordance with the present invention.
Fig. 9 shows TEM image for a longitudinal ITO-tin oxide heterostructure nanowires.
Fig. 10 shows the line element profile of longitudinal ITO-tin oxide heterostructure nanowires
Fig. 11 shows Mapping image for longitudinal ITO-tin oxide heterostructure nanowires.
Fig 12 show In-situ XRD analysis of longitudinal ITO-tin oxide heterostructure nanowires finally obtained using oxidation process of lateral heterostructure nanowires having indium/tin core and graphitic shell in accordance with the present invention.
Fig. 13 shows In-situ Raman' analysis of longitudinal ITO-tin oxide heterostructure nanowires finally obtained using oxidation process of lateral heterostructure nanowires having indium/tin core and graphitic shell in accordance with the present invention.
Fig. 14 shows the result of superconducting properties analysis of lateral heterostructure nanowires having indium/tin core and graphitic shell in accordance with the present invention.
Fig. 15 shows lateral heterostructure nanowires having bismuth/tin core and graphitic shell synthesized in the same manner as the present invention.
Fig 16 show measurement result of CL (cathodoluminescence) of longitudinal ITO-tin oxide heterostructure nanowires.
Fig. 17 shows SEM image for reversible synthesis to lateral heterostructure nanowires having indium/tin core and graphitic shell of longitudinal ITO-tin oxide heterostructure nanowires.

### DETAILED DESCRIPTION

As described below, the synthesis method of graphitic shell-alloy core heterostructure nanowires and longitudinal metal oxide heterostructure nanowires and a reversible synthesis method thereof in the invention will described with reference to the accompanying drawings.

The present invention to achieve the above noted object provides a synthesis method of lateral heterostructure nanowires containing alloy core and graphitic shell, according to claim 1.

In addition, the present invention to achieve the above noted object provides a synthesis method of longitudinal metal oxide heterostructure nanowires wherein, according to claim 2.

Furthermore, the present invention to achieve the above noted object provides a reversible synthesis method between graphitic shell-alloy core heterostructure nanowires and longitudinal metal oxide heterostructure nanowires, according to claim 3.

Referring now to Fig.1, the process for forming heterostructure nanowires are described in detail. First, lateral heterostructure nanowires based on a graphitic shell is synthesized to synthesize a longitudinal heterostructure nanowires comprised of at least two kinds of substances in its growth direction.

A metal oxide serves as catalyst that can produce graphitic shell to synthesize lateral heterostructure nanowires based on graphitic shell should be prepared, wherein, the choice of metal oxide is made according to whether the product generated after the metal oxide is reduced has a catalytic activity adapted to synthesize carbon. Even if there is various metal oxides having a catalyst activity, indium oxide and tin oxide are described for clear description in the embodiments described below,

First, the prepared indium oxide and tin oxide are soaked in distilled water. At this point, the rate of tin oxide to indium oxide is regulated in the range of 6:1∼1:6 based on a weight rate, and the weight of the entire mixture of metal oxides in the distilled water is regulated within 10wt% of the distilled water weight.

So aqueous solution of prepared metal oxides is uniformly mixed using a magnetic bar rotating at 200rpm for 10∼30 minute and then only the metal oxide particles is selectively recovered using cellulose filter with pores of 200nm size filled with an uniformly maxed oxide aqueous.

Next, the recovered metal oxide is placed in the oven set at 100°C and is dried to completely remove the residual moisture in the surface of said recovered metal oxide, so a preparation of metal oxide mixture for synthesizing heterostructure nanowires is finished.

And then a quartz boat is filled with dried metal oxide mixture to synthesize heterostructure nanowires from next prepared metal oxide and then the mixture is placed in a inner portion of a prepared reactor and a degree vacuum of internal reactor is decreased to a maximum 10⁻²Torr while removing all a residual oxygen prior to a start of synthesis.

When a vacuum work is finished, a vacuum pump is turn off, and a temperature of a reactor is increased to the rang of 550∼850 °C adapted to a synthesis while a gas such as argon or nitrogen serving as a carrier gas is supplied.

When the temperature of a reactor is increased to a synthesis temperature, hydrocarbon gas which is carbon source is provided. Any one or more than two of acetylene, methane and ethylene may be used as hydrocarbon gas, and the amount of hydrocarbon flowing into said reactor is preferably in the range of 2∼10 vol%. The supplied gas is first decomposed into carbon and hydrogen on the surface of metal oxide particles positioned in the boat of the inner portion of the reactor.

At this time, the decomposed hydrogen element serves to reduce metal oxide such as indium oxide and tin oxide. That is, in process that indium oxide and tin oxide are gradually reduced as metal indium and metal tin from the surface, resulting in the production of alloy of indium and tin or intermetallic nanoparticles.

This is possible because the melting point of indium and tin which is in 153°C and 231°C, and eutectic temperature of their alloy is below 200 °C, or so is lower than synthesis temperature of 550∼850 °C. Nanoparticles comprised of reduced indium and tin serve to perform catalyst role forming graphitic shell that is, crystallized carbon structure having carbon atoms decomposed by catalyst reaction therein.

In this process, graphitic shell may act as one container and continue to be formed and indium/tin solution form nanowires while being continued to move along graphitic shell.

As a result, such a growth mechanism enables to form heterostructure involving intermetallic or alloys core filled with indium and tin therein and graphitic shell. At this time, the synthesis time is preferably performed up to 2 hours.

On the other hand, in said synthesis process, small quantities of hydrogen may be added into a reactor to more prompt the reduction of metal oxide and to suppress a generation of amorphous carbon.

If hydrogen is too many, the reduction of metal oxide is too fast and therefore, the production of intermetallic or alloy of indium and tin is too precipitated.

Therefore, heterostructure nanowires become too large in size and synthetic yield of hetero nanowires can be degraded, whereby the supply amount of hydrogen is preferably 0∼5Vol%.

When this synthesis is finished, the temperature of a reactor is cooled to a room temperature under a carrier gas atmosphere and then lateral heterostructure nanowires based graphitic shell produced is obtained. In this way, the synthesis of lateral heterostructure nanowires comprised of graphitic shell and indium/tin core is primarily finished.

As a result, it can be confirmed that lateral heretostructure nanowires having indium/tin and graphitic shell synthesized by the present application is 50∼150 nm in a diameter, thickness of graphitic shell is 1∼20nm and the length is 1∼10*µ*m.

The lateral core-shell heterostructure nanowires obtained after this is placed into quartz or aluminum boat and the oxidation process is started.

The oxidation temperature is preferably 350∼650°C, in which the most of substance used as core in graphitic shell can be converted into metal oxides.

The rise of temperature is preferably 1∼10°C/min, in which the abrupt temperature rise allows an abrupt incineration of graphitic shell and the oxidation speed of core substance to be too fast, and thus cannot keep a desirable type of nanowires.

The time of the oxidation processing is performed in range of 1 minute ∼ 6 hours and the heat processing atmosphere gas is preformed in a general air atmosphere, thereby making it to provide an additional air. When the oxidation process is finished, in case the temperature of reactor is cooled to a room temperature and the sample is obtained, the synthesis of longitudinal ITO-tin oxide heterostructure nanowires is finished.

The lateral heretostructure nanowires are incinerated by the reaction with oxygen through the above-mentioned oxidation processing. The incineration speed may be controlled based on a temperature rising rate of reactor, and an oxidation reaction processing time and an oxygen density control, which is a very important control factor.

An intermetallics or alloy of indium/tin in graphitic shell is in solution, which is converted into oxides by contacting with oxygen along with progressive incineration of graphitic shell.

In this process, an intermetallics or alloy of indium/tin again is divided into two. Two oxides are maintained in form of nanowires and thus longitudinal ITO-tin oxide heterostructure nanowires are synthesized.

It can be confirmed that longitudinal ITO-tin oxide heterostructure nanowires are in the range of 50∼150nm in a average diameter, is formed preferably in 100nm and the length is 1∼10*µ*m.

In addition, longitudinal ITO-tin oxide heterostructure nanowires can be again converted into the lateral heterostructure nanowires comprised of an intermetallics or a alloy core-graphitic shell using a above-mentioned supply method. Therefore, it can be shown that the reversible synthesis between graphitic shell-intermetallics or alloys core heterostructure nanowires and longitudinal ITO-tin oxide heterostructure nanowires become possible.

As described below, an embodiment will be described in regard to the synthesis method for graphitic shell-alloys core heterostructure nanowires and longitudinal metal oxide nanowires. However, the scope of the present invention is not limited to the preferable embodiment, and those skilled in the art will be appreciated to understand various modified form of disclosure described in the specification.

### [Embodiment 1] XRD graph for lateral heterostructure nanowires produced according to weight rate of tin oxide and indium oxide

Fig.2 shows XRD graph for lateral heterostructure nanowires having indium/tin intermetallic core and graphitic shell in accordance with the present application

The difference for heterostructure nanowires produced according to a weight rate of tin oxide and indium oxide in the embodiment was interpreted using XRD analysis.

It can be confirmed that if tin oxide:indium oxide is 6:1, intermetallics of InSn₄ composed of the rate that tin is 4 and indium is 1 is produced.

It could be confirmed that as the rate of indium oxide in mixture of tin oxide and indium oxide increase, a intermetallics of In₃Sn composed of the rate that tin is 1 and indium 3, along with InSn₄ is produced, and it could be shown that if tin oxide; indium oxide is 1:6, indium/tin core is positioned in the inner portion of graphitic shell appears mostly as In₃Sn.

### [Embodiment 2] SEM image according synthesis temperature

Fig.3 shows SEM image according to the synthesis temperature of lateral heterostructure nanowires having indium/tin intermetallic core and graphitic shell in accordance with the present application, in which (a), (b), (c) and (d) illustrate SEM image for heterostructure nanowires synthesized at 550, 650, 750 and 850°C, respectively.

It was confirmed that heterstructure nanowires are partially produced at 550 °C of the synthesis and, it could be known that a synthesis yield of heterostructure nanowires are increased considerably. Such a tendency was appear as more remarkable phenomenon.

In particular, it can be confirmed that graphitic shell surrounding indium/tin core which is contained in the inner portion thereof and the outer portion is clearly exist.

However, if the synthesis temperature is increased to 850 °C, it could be confirmed that a yield of heterostructure nanowires decreased, whereas, a diameter of heterostructure nanowires considerably increased. Finally, it was confirmed that a diameter of heterostructure nanowire increased according to increase of synthesis temperature and the highest yield is favorably obtained at 650∼750°C.

### [Embodiment 3] SEN image for core-shell heterostructure nanowires produced according to synthesis time

Fig.4 shows SEM image according to synthesis time of heterostructure nanowires having indium/tin intermetallic core and graphitic shell in accordance with the present application, in which (a), (b), (c) and (d) illustrate SEM image for heterostructure nanowires synthesized at 1, 5, 10 and 60 minute, respectively.

It was confirmed that the product synthesized for 1 minute exist as particle phase and it was appeared that these particles are mixed with indium oxide and tin oxide which is not reduced yet, partially reduced indium and tin as well as alloy of indium/tin.

If a synthesis time is increased to 5 minute, the appearance was partially observed, and the produced nanowires are short yet and the yield is less and particles that is considered as indium oxide and tin oxide which is not reduced yet, partially reduced indium and tin as well as alloy of indium/tin were observed.

If a synthesis time is increased to 10 minute, it was observed that hetero structure nanowires are at most of surface, the existence of indium oxide and tin oxide was confirmed as a minute amount, and what indium oxide and tin oxide are converted into indium/tin intermetallics nanowires was almost observed using SEM image.

Such a result is supported by XRD graph for associated product. It was confirmed that the length of produced heterostructure nanowires is above 5*µ*m.

### [Embodiment 4] TEM image of the produced core-shell heterostructure nanowires

Fig.5 shows TEM image according to the synthesis time of heterostructure nanowires having indium/tin intermetallic core and graphitic shell in accordance with the present application
(a) is a low magnification image of the heterostructure nanowires, in which it was confirmed that a core is enclosed by graphitic shell and it was confirmed that core/ tin core within graphitic shell is filled above 90%.

It was confirmed that the lattice structure of core included through a high magnification TEM image (b) is intermetallics of indium/tin

And, it was confirmed that this is InSn₄ or In₃SN depending on mixture rate of tin oxide and indium oxide as shown in Fig. 2. In addition, lattice spacing of the core was calculated to 0.34 nm.

### [Embodiment 5] Component analysis for the produced core-shell heterostructure nanowires

Fig.6 shows the element analysis of heterostructure nanowires having indium/tin intermetallic core and graphitic shell in accordance with the present application.

As shown in the drawing, it was conformed that component of shell is carbon and the core that is contained in the inner portion of the shell is component containing indium and tin.

It was confirmed that because such a result completely corresponds to the above mentioned TEM image, the shell of heterostructure nanowires is a nanotube that resembles CNT, and the core is the intermetallics comprised of indium and tin.

The heterostructure nanowires shown in drawing of the embodiment was confirmed that InSn₄ intermetallics contained at the rate that indium is 1 and tin is 4 is produced as a core.

### [Embodiment 6] XRD graph for longitudinal ITO-tin oxide heterostructure nanowires

Fig 7 show XRD graph for longitudinal ITO-tin oxide heterostructure nanowires in the present invention.

As-received illustrates XRD graphy for a mixture of indium oxide and tin oxide, and 1ₛₜ synthesis is a XRD graph obtained by reacting the mixture of indium oxide and tin oxide with acetylene at 750°C for 1 hour, It can be confirmed from InSn₄ and In₃Sn which the intermetallics are produced in said graph.

It can be confirmed that the graphitics shell is fully removed by the oxidation processing for the produced indium/tin core-graphitic shell heterostructure nanowires at 650°C and it can be confirmed that the oxidized product is crystal structure that is similar to that of indium oxide and tin oxide of As-received which is original sample. Specifically, it can be confirmed that ITO that tin oxide is partially contained in indium oxide.

### [Embodiment 7] SEM image for the produced longitudinal ITO-tin oxide heterostructure nanowires

Fig. 8 shows SEM image for longitudinal ITO-tin oxide heterostructure nanowires obtained using oxidation process of lateral heterostructure nanowires having indium/tin core and graphitic shell in accordance with the present invention.

The drawing illustrates the longitudinal ITO-tin oxide heterostructure nanowires obtained from the oxidation treatment for the primarily synthesized lateral heterostructure nanowires. Even if the its size look similar to the primarily synthesized core-shell heterostructure nanowires at 650°C, the its presence was not conformed and it was observed that some nano particle is partially on the surface of the nanowire. In addition, it was also observed that the boundary layer is in the middle of the middle.

### [Embodiment8] TEM image for produced indium/tin mixture- tin oxide hetero nano wires

Fig. 9 shows TEM image for a longitudinal ITO-tin oxide heterostructure nanowires.
(a) illustrates a low magnification of longitudinal ITO-tin oxide heterostructure nanowires produced by the oxidation treatment of the lateral heterostructure nanowires at 650°C, where, the graphitic shell is not observed in its outer portion, and it was confirmed that the layer in which the substance having a different contrast in the middle of nanowires generate is formed.

STEM image of (b) shows clearly such the difference in a contrast. Since a difference in contrast has an different specific gravity for each substance, it was confirmed in the structure in which the different substance is connected each other. (c) is the image for the high magnification of (a) and, (d) shows XRD diffraction pattern for an upper end and an lower end based on the boundary of (c). According to the analysis for each diffraction pattern, it was clearly confirmed that the lower end is ITO and the upper end is tin oxide.

### [Embodiment 9] EXD analysis for the produced longitudinal ITO-tin oxide heterostructure nanowires

Fig. 10 shows the line element profile of longitudinal ITO-tin oxide heterostructure nanowires.
(a) is TEM image, in which the boundary was confirmed in the middle of nanowires, and drawing (b) shows the line profile for STEM image of (a) and the associated component, confirmed that there is indium, tin, and oxygen in the lower end and tin and oxygen in the upper. This can confirm that ITO is formed in the lower end and tin oxide is formed in the upper end.

### [Embodiment 10] STEM and Mapping for the produced longitudinal ITO-tin oxide heterostructure nanowires

Fig. 11 shows Mapping image for longitudinal ITO-tin oxide heterostructure nanowires.

One nanowire can be observed in the STEM image, wherein the mapping image of the entire components relative to thereof is shown in Drawing (c) to (e). (c) is indium, (d) is tin, and (e) is oxygen component.

As a result, oxygen was confirmed in the whole portion of nanowire for analysis. However, it was confirmed that there are indium and tin along the longitudinal direction. Especially, the small amount of tin was detected.

Such a result could clearly confirm in the overlay area (c). This clearly shows that the produced nanowires are ITO-tin oxide heterostructure nanowires formed in longitudinal direction.

### [Embodiment 11] In-suit XRD for longitudinal ITO-tin oxide heterostructure nanowires obtained finally using oxidation treatment of the lateral heterostructure nanowires having indium/tin core and graphitic shell.

Fig 12 show In-situ XRD analysis result of longitudinal ITO-tin oxide heterostructure nanowires finally obtained using oxidation process of the lateral heterostructure nanowires having indium/tin core and graphitic shell in accordance with the present invention.

It be should noted that the measurement was made while the temperature increases from 20°C to 650°C.

In up to 120°C, IN₃Sn and InSn₄ relative to intermetallics of indium and tin was observed. However, in more than 120 to 350°C, No the phase was found. This means that intermetallics of indium and tin are at liquid state. In actual, there is the melting point of intermetallics of indium and tin according to the component at 120 to 220°C. After this, from 350 °C, the phase relative to indium oxide and tin mixture was observed at first, and it was confirmed that as the temperature approaches to 650°C, the phase appears more greater. This shows that intermetallics of indium and tin of the liquid phase in graphitic shell is converted gradually into the metal oxide form.

### [Embodiment 12] In-situ Raman for longitudinal ITO-tin oxide heterostructure nanowires finally obtained using oxidation process of the lateral herterostructure nanowires having indium/tin core and graphitic shell

Fig. 13 shows In-situ Raman' analysis for longitudinal ITO-tin oxide heterostructure nanowires finally obtained using oxidation process of the lateral heterostructure nanowires having indium/tin core and graphitic shell in accordance with the present invention.

It be should noted that the measurement was made while the temperature increases from 20 to 600°C.

The Raman spectra show that of the same result of XRD. Only D-band and G-band related to graphitic shell was confirmed in Raman spectra of the low temperature. In actual, the intermetallics of indium and tin were not exited. Therefore, it is natural that such result was derived between intermetallic core of indium and tin, and core-shell heterostructure nanowires. However, D-band and G band corresponding to graphitic shell gradually disappears as increase of temperature, and peaks of the metal oxide related to tin and indium were found. Especially, The most significant measured peck at 150 to 200cm⁻¹ among especially indium related peaks shows a shape in which is confirmed in ITO that a small amount of tin is mixed with indium oxide. These results shows that the lateral heterostructure nanowire having indium/tin core and graphitic shell using oxidation process of the high temperature can be converted into longitudinal ITO-tin oxide heterostructure nanowires.

### [Embodiment 13] Superconducting properties analysis for the produced lateral heterostructure nano wires

Fig. 14 shows the result of superconducting properties analysis of the lateral heterostructure nanowires having indium/tin core and graphitic shell in accordance with the present invention.

In Figure 14, it was conformed that the magnetization characteristic according to the temperature of the produced lateral heterostructure nanowires shows the same tendency as the superconductor characteristic. In addition, the bulk superconductor temperature was determined at 4.8∼6.0 K, and it was conformed that this is higher than the superconductor temperature of pure tin (T_{c}=3.7K). It was confirmed that the different superconductor temperature is shown according to the rate of indium and tin of herterostructure nanowires having such indium/tin core.

In view the above-mentioned results, heterostructure nanowires produced according to the present invention may be utilized as a useful superconductor material.

### [Embodiment 14] lateral heterostructure nanowires synthesis using bismuth oxide and tin oxide, not according to the invention.

Fig. 15 shows lateral heterostructure nanowires having bismuth/tin core and graphitic shell synthesized in the same manner as the present invention.

The synthesis method was performed as described in the above embodiments and Fig.1.
(a) shows SEM image for lateral heterostructure nanowires having produced bismuth /tin core and graphitic shell.

The synthesized form is similar to indium/tin core-graphitic shell heterostructure nanowires, and it was confirmed that bismuth/tin core is contained above 90% in the inside of graphiticl.

A low magnification and a high magnification TEM images (b) and (c) of said synthesized lateral heterostructure nanowires, and component analysis (d) clearly was shown that synthesized heterostructure nanowires are made of bismuth/tin alloy in the inner space of graphitics shell.

### [Embodiment 15] The CL measurement result for longitudinal ITO-tin oxide heterostructure nanowires

Fig 16 show measurement result of CL (cathodoluminescence) of longitudinal ITO-tin oxide heterostructure nanowires

It was shown that the SEM image of (a) has the longitudinal ITO-tin oxide heterostructure nanowires. The difference in brightness was partially observed clearly in view of the measured result of CL characteristic for such heterostructure nanowires. This also shows a portion of ITO in which the energy bandgap is relatively large looks brighter than in the part of tin oxide. Therefore, it is demonstrated that the nanowires are longitudinal ITO-tin oxide heterostructure nanowires.

### [Embodiment 16] Reversible synthesis to lateral heterostructure nanowires having indium/tin core and graphitic shell of longitudinal ITO-tin oxide heterostructure nanowires

Fig. 17 shows SEM image for reversible synthesis to lateral heterostructure nanowires having indium/tin core and graphitic shell of longitudinal ITO-tin oxide heterostructure nanowires.
(a) shows the lateral heterostructure nanowires having indium/tin core and graphitics shell synthesized through the primarily synthesized core-shell hetero structure nanowires synthesis process. (b) shows the longitudinal ITO-tin oxide heterostructure nanowires synthesized through 650° oxidation process for the primarily synthesized core-shell heterostructure nanowires and (c) shows the lateral herterostructure nanowires having indium /tin core and graphitic shell synthesized through the reversible process appliable again longitudinal ITO-tin oxide heterostructure nanowires to the primary core-shell heterostructure nanowires. As a result, it was confirmed that the lateral heterostructure nanowires having indium/tin core and graphitic shell and longitudinal ITO-tin oxide heterostructure nanowires make the reversible synthesis possible each other.

As described above, after synthesizing lateral heterostruccture nanowires comprised of graphitic shell and intermetllics or alloy core as a medium of metal oxide mixture and oxdizes it to remove the graphitic shell on the surface and oxidizes and separates intermetallics or alloy to synthesize the novel type of longitudinal metal oxide heterostructure wires.

Using such principle, the lateral heterostructure nanowires are synthesized using simultaneously the various substance and longitudinal heterostructure nanowires containing various substance can be produced in volume as a very simple process.

While the described embodiment represents the preferred form of the prevent invention, it is to be understood that modifications will occur to those skilled in the art without departing from the scope of the appended claims.

## Claims

1. A synthesis method of lateral heterostructure nanowires containing an alloy core and a graphitic shell having a superconducting critical temperature (Tc) in the range of 4.8∼6.0 K, the method comprised of:
i) a step for preparing a metal oxide mixture, installing it into a reactor, and supplying a carrier gas under a vacuum atmosphere to increase the internal temperature of the reactor to the synthesis temperature,
ii) a step for supplying hydrocarbon gas into said reactor and reacting said gas with said metal oxide mixture;
wherein said metal oxide mixture is a mixture of indium oxide and tin oxide, and said mixture rate of said indium oxide and tin oxide is 6:1∼1:6 based on a weight rate.

2. A synthesis method of longitudinal heterostructure nanowires containing metal oxides along the longitudinal direction, the method comprised of:
i) a step for preparing a metal oxide mixture, installing it into an reactor, and supplying an carrier gas under a vacuum atmosphere to increase the internal temperature of a reactor to a synthesis temperature,
ii) a step for supplying hydrocarbon gas into said reactor and reacting the gases with said metal oxide mixture to synthesize lateral heterostructure nanowires containing an alloy core and a graphitic shell,
iii) a step cooling said reactor to a room temperature, and increasing again the temperature under an oxide atmosphere to oxidize the lateral heterostructure nanowires containing an alloy core and a graphitic shell;
wherein said metal oxide mixture is a mixture of indium oxide and tin oxide, and said mixture rate of said indium oxide and tin oxide is 6:1∼1:6 based on a weight rate.

3. A reversible synthesis method between graphitic shell-alloy core heterostructure wires and longitudinal metal oxide heterostructure nanowires containing metal oxides along the longitudinal direction, the method comprised of:
i) a step for reacting a metal oxide mixture and hydrocarbon gases within a reactor to synthesize lateral heterostructure nanowires having an alloy core and a graphitic shell, and
ii) a step for oxidizing lateral heterostructure nanowires of said synthesized core-shell to synthesize longitudinal metal oxide heterostructure nanowires containing metal oxides along the longitudinal direction,
and said step i) and ii) are performed repeatedly;
wherein said metal oxide mixture is a mixture of indium oxide and tin oxide, and said mixture rate of said indium oxide and tin oxide is 6:1∼1:6 based on a weight rate.

4. The synthesis method of claim 1 to 3, wherein:
said hydrocarbon gas flowing into said reactor is a one or more selected from acetylene, ethylene and methane or a mixture thereof, and the amount of hydrocarbon gas flowing into said reactor is in the range 2∼10 vol% based on said carrier gas.

5. The synthesis method of claim 1 to 3, wherein:
hydrogen gas is flown into said reactor to assist the reaction of said metal oxide mixture and hydrocarbon, and the inflow amount of said hydrogen gas is less than 5 vol%.

6. The synthesis method of claim 1 to 3, wherein:
a reaction temperature of said metal mixture oxide and hydrocarbon gas is controlled in the range of 550∼850°C, and a reaction time is within 2 hours.

7. The synthesis method of claim 2 to 3, wherein:
an oxidation processing temperature of said graphitic shell-alloy core heterostructure nanowires is controlled in the range of 350∼650°C, and an oxidation processing time is 1 minute ∼6hours.

8. The synthesis method of claim 2 to 3, wherein:
a temperature rise for oxidation processing of said graphitic shell-alloy core heterostructure nanowires is obtained at 1∼10°C/min.

9. A lateral heterostructure nanowire containing an alloy core and graphitic shell synthesized by the synthesis of any one of claims 1, 3 and claim 4 to 6, wherein the alloy is a mixture of indium and tin, and said mixture rate of said indium and tin is 6:1∼1:6 based on a weight rate, wherein the diameter is 50∼150nm, and the length is 100nm∼10µm, and the thickness of said shell is 1∼20nm, and said alloy is filled in more than 90% of the inner portion of said graphitic shell, wherein a superconducting critical temperature (Tc) in the range of 4.8-6.0 K is determined.

10. A longitudinal heterostructure nanowire containing metal oxides along the longitudinal direction synthesized by a method of any one of claims 2, 3 and claim 4 to 8, wherein said metal oxide mixture is a mixture of indium oxide and tin oxide, and said mixture rate of said indium oxide and tin oxide is 6:1∼1:6 based on a weight rate, wherein the average diameter is in the range of 50∼150nm, and the length is 100nm∼10µm.

## Patentansprüche

1. Syntheseverfahren von Nanodrähten mit lateraler Heterostruktur, die einen Legierungskern und eine Graphithülle enthalten, und die einen supraleitenden kritischen Temperaturbereich (Tc) im Bereich von 4,8∼6,0 K aufweisen, wobei das Verfahren folgende Schritte aufweist:
i) einen Schritt zur Präparation einer Metalloxidmischung, zum Einführen dieser in einen Reaktor, und zum Zuführen eines Trägergases unter einer Vakuumatmosphäre, um die interne Temperatur des Reaktors auf die Synthesetemperatur zu erhöhen,
ii) einen Schritt zum Zuführen von Kohlenwasserstoffgas in den Reaktor und Reagieren des Gases mit der Metalloxidmischung;
wobei die Metalloxidmischung eine Mischung aus Indiumoxid und Zinnoxid ist, und wobei das Mischungsverhältnis des Indiumoxids und des Zinnoxids, basierend auf einem Gewichtsverhältnis, 6:1 ∼ 1:6 beträgt.

2. Syntheseverfahren von Nanodrähten mit länglicher Heterostruktur, die Metalloxide entlang der Längsrichtung enthalten, wobei das Verfahren die folgenden Schritte aufweist:
i) einen Schritt zur Präparation einer Metalloxidmischung, zum Einführen dieser in einen Reaktor, und zum Zuführen eines Trägergases unter einer Vakuumatmosphäre, um die interne Temperatur eines Reaktors auf eine Synthesetemperatur zu erhöhen,
ii) einen Schritt zum Zuführen von Kohlenwasserstoffgas in den Reaktor und Reagieren des Gases mit der Metalloxidmischung, um Nanodrähte mit lateraler Heterostruktur, die einen Legierungskern und eine Graphithülle aufweisen, zu synthetisieren,
iii) einen Schritt zum Kühlen des Reaktors auf Raumtemperatur, und zum erneuten Erhöhen der Temperatur unter einer Oxidatmosphäre, um die Nanodrähte mit lateraler Heterostruktur, die einen Legierungskern und eine Graphithülle aufweisen, zu oxidieren;
wobei die Metalloxidmischung eine Mischung aus Indiumoxid und Zinnoxid ist, und wobei das Mischungsverhältnis des Indiumoxids und des Zinnoxids, basierend auf einem Gewichtsverhältnis, 6:1 ∼ 1:6 beträgt.

3. Reversibles Syntheseverfahren zwischen Drähten mit Graphithüllenlegierungskernheterostruktur und Nanodrähten mit länglicher Metalloxidheterostruktur, die Metalloxide in der Längsrichtung aufweisen, wobei das Verfahren die folgenden Schritte aufweist:
i) einen Schritt zum Reagieren einer Metalloxidmischung und Kohlenwasserstoffgasen in einem Reaktor, um Nanodrähte mit lateraler Heterostruktur, die einen Legierungskern und eine Graphithülle aufweisen, zu synthetisieren, und
ii) einen Schritt zum Oxidieren von Nanodrähten mit lateraler Heterostruktur der synthetisierten Kernhülle, um Nanodrähte mit länglicher Metalloxidheterostruktur, die Metalloxide in der Längsrichtung aufweisen, zu synthetisieren;
und die Schritte i) und ii) werden wiederholt ausgeführt;
wobei die Metalloxidmischung eine Mischung aus Indiumoxid und Zinnoxid ist, und wobei das Mischungsverhältnis des Indiumoxids und des Zinnoxids, basierend auf einem Gewichtsverhältnis, 6:1 ∼ 1:6 beträgt.

4. Syntheseverfahren nach Anspruch 1 bis 3, wobei:
das Kohlenwasserstoffgas, das in den Reaktor strömt, eines oder mehrere ist, die aus einer Gruppe ausgewählt ist, die aus Acetylen, Ethylen und Methan, oder einer Mischung davon besteht, und die Menge des Kohlenwasserstoffgases, das in den Reaktor strömt, basierend auf dem Trägergas, im Bereich von 2 ∼ 10 vol % liegt.

5. Syntheseverfahren nach Anspruch 1 bis 3, wobei:
Wasserstoffgas in den Reaktor eingeleitet wird, um die Reaktion der Metalloxidmischung und dem Kohlenwasserstoff zu unterstützen, und die Einleitmenge des Wasserstoffgases geringer als 5 vol % ist.

6. Syntheseverfahren nach Anspruch 1 bis 3, wobei:
eine Reaktionstemperatur der Metalloxidmischung und des Kohlenwasserstoffgases im Bereich von 550 ∼ 850°C gesteuert wird, und eine Reaktionszeit innerhalb von 2 Stunden liegt.

7. Syntheseverfahren nach Anspruch 2 bis 3, wobei:
eine Oxidationsaufbereitungstemperatur der Nanodrähte mit Graphithüllenlegierungskernheterostruktur im Bereich von 350-650°C gesteuert wird, und eine Oxidationsaufbereitungszeit zwischen 1 Minute und 6 Stunden liegt.

8. Syntheseverfahren nach Anspruch 2 bis 3, wobei:
ein Temperaturanstieg für die Oxidationsaufbereitung der Nanodrähte mit Graphithüllenlegierungskernheterostruktur bei 1 ∼ 10°C/min erhalten wird.

9. Nanodraht mit lateraler Heterostruktur, der einen Legierungskern und eine Graphithülle aufweist, und der durch die Synthese nach einem der Ansprüche 1, 3 und der Ansprüche 4 bis 6 synthetisiert wurde, wobei die Legierung eine Mischung aus Indium und Zinn ist, und wobei das Mischungsverhältnis des Indiums und des Zinns, basierend auf einem Gewichtsverhältnis, 6:1 ∼ 1:6 beträgt, wobei der Durchmesser 50 ∼ 150nm beträgt, und die Länge 100 nm ∼ 10 µm beträgt, und die Dicke der Hülle 1 ∼ 20 nm beträgt, wobei die Legierung in mehr als 90 % des inneren Abschnitts der Graphithülle gefüllt ist, wobei ein supraleitender kritischer Temperaturbereich (Tc) im Bereich von 4,8 ∼ 6,0 K festgelegt ist.

10. Nanodraht mit länglicher Heterostruktur, der Metalloxide in der Längsrichtung aufweist, und der durch ein Verfahren nach einem der Ansprüche 2, 3 und der Ansprüche 4 bis 8 synthetisiert wurde, wobei die Metalloxidmischung eine Mischung aus Indiumoxid und Zinnoxid ist, wobei das Mischungsverhältnis des Indiumoxids und des Zinnoxids, basierend auf einem Gewichtsverhältnis, 6:1 ∼ 1:6 beträgt, und wobei der durchschnittliche Durchmesser im Bereich von 50 ∼ 150 nm und die Länge im Bereich von 100 nm ∼ 10 µm liegt.

## Revendications

1. Procédé de synthèse de nano-fils d'hétérostructure latérale contenant un coeur d'alliage et une enveloppe graphitique ayant une température critique de supraconduction (Tc) dans la plage comprise entre 4,8 et 6,0 K, le procédé comprenant :
i) une étape de préparation d'un mélange d'oxydes métalliques, de sa mise en place dans un réacteur, et d'alimentation d'un gaz porteur en atmosphère sous vide pour augmenter la température interne du réacteur à la température de synthèse,
ii) une étape d'alimentation d'un gaz hydrocarbure dans ledit réacteur et de mise en réaction dudit gaz avec ledit mélange d'oxydes métalliques,
dans lequel ledit mélange d'oxydes métalliques est un mélange d'oxyde d'indium et d'oxyde d'étain, et dans lequel ledit rapport de mélange desdits oxyde d'indium et oxyde d'étain est compris entre 6 : 1 et 1 : 6, sur la base d'un rapport de poids.

2. Procédé de synthèse de nano-fils d'hétérostructure longitudinale contenant des oxydes métalliques le long de la direction longitudinale, le procédé comprenant :
i) une étape de préparation d'un mélange d'oxydes métalliques, de sa mise en place dans un réacteur, et d'alimentation d'un gaz porteur en atmosphère sous vide pour augmenter la température interne d'un réacteur à une température de synthèse,
ii) une étape d'alimentation d'un gaz hydrocarbure dans ledit réacteur et de mise en réaction des gaz avec ledit mélange d'oxydes métalliques pour synthétiser des nano-fils d'hétérostructure latérale contenant un coeur d'alliage et une enveloppe graphitique,
iii) une étape de refroidissement dudit réacteur à une température ambiante, et de nouvelle augmentation de la température sous une atmosphère d'oxyde pour oxyder les nano-fils d'hétérostructure latérale contenant un coeur d'alliage et une enveloppe graphitique,
dans lequel ledit mélange d'oxydes métalliques est un mélange d'oxyde d'indium et d'oxyde d'étain, et ledit rapport de mélange dudit oxyde d'indium et d'oxyde d'étain est de 6 : 1 à 1 : 6, sur la base d'un rapport de poids.

3. Procédé de synthèse réversible entre des fils d'hétérostructure coeur d'alliage-enveloppe graphitique et des nano-fils d'hétérostructure d'oxydes métalliques longitudinale contenant des oxydes métalliques le long de la direction longitudinale, le procédé comprenant :
i) une étape de mise en réaction d'un mélange d'oxydes métalliques et de gaz hydrocarbures dans un réacteur pour synthétiser des nano-fils d'hétérostructure latérale ayant un coeur d'alliage et synthétisés, et
ii) une étape d'oxydation de nano-fils d'hétérostructure latérale dudit coeur-enveloppe synthétisé pour synthétiser des nano-fils d'hétérostructure d'oxydes métalliques longitudinale contenant des oxydes métalliques le long de la direction longitudinale,
et dans lequel lesdites étapes i) et ii) sont réalisées de manière répétée,
dans lequel ledit mélange d'oxydes métalliques est un mélange d'oxyde d'indium et d'oxyde d'étain, et ledit rapport de mélange desdits oxyde d'indium et oxyde d'étain compris entre 6 : 1 et 1 : 6, sur la base d'un rapport de poids.

4. Procédé de synthèse des revendications 1 à 3, dans lequel :
ledit gaz hydrocarbure qui s'écoule dans ledit réacteur est un ou plusieurs gaz choisi (s) dans l'acétylène, l'éthylène et le méthane ou un mélange de ceux-ci, et la quantité de gaz hydrocarbure qui s'écoule dans ledit réacteur est dans la plage de 2 à 10 % en volume, sur la base dudit gaz porteur .

5. Procédé de synthèse des revendications 1 à 3, dans lequel :
le gaz hydrogène est envoyé dans ledit réacteur pour faciliter la réaction dudit mélange d'oxydes métalliques et de l'hydrocarbure, et la quantité d'apport dudit gaz hydrogène est inférieure à 5 % en volume.

6. Procédé de synthèse des revendications 1 à 3, dans lequel :
une température de réaction dudit mélange d'oxydes métalliques et de gaz hydrocarbure est contrôlée dans la plage de 550 à 850°C, et dans lequel un temps de réaction est de +/- 2 heures.

7. Procédé de synthèse des revendications 2 à 3, dans lequel :
une température de traitement d'oxydation desdits nano-fils d'hétérostructure coeur d'alliage-enveloppe graphitique est contrôlée dans la plage de 350 à 650°C, et dans lequel un temps de traitement d'oxydation est compris entre 1 minute et 6 heures.

8. Procédé de synthèse des revendications 2 à 3, dans lequel :
une augmentation de température pour le traitement d'oxydation desdits nano-fils d'hétérostructure coeur d'alliage-enveloppe graphitique est obtenue entre 1 et 10°C / min.

9. Nano-fil d'hétérostructure latérale contenant un coeur d'alliage et une enveloppe graphitique synthétisés par la synthèse de l'une quelconque des revendications 1, 3 et des revendications 4 à 6, dans lequel l'alliage est un mélange d'indium et d'étain, et dans lequel ledit rapport de mélange desdits indium et étain est de 6 : 1 à 1 : 6, sur la base d'un rapport de poids, dans lequel le diamètre est compris entre 50 et 150 nm, et la longueur est comprise entre 100 nm et 10 µm, et l'épaisseur de ladite enveloppe est comprise entre 1 et 20 nm, et ledit alliage est rempli, dans plus de 90 % de la partie intérieure, de ladite enveloppe graphitique dans laquelle une température critique de supraconduction (Tc), dans la plage comprise entre 4,8 et 6,0 K, est déterminée.

10. Nano-fil d'hétérostructure longitudinale contenant des oxydes métalliques le long de la direction longitudinale, synthétisés par un procédé de l'une quelconque des revendications 2, 3 et des revendications 4 à 8, dans lequel ledit mélange d'oxydes métalliques est un mélange d'oxyde d'indium et d'oxyde d'étain, et dans lequel ledit rapport de mélange desdits oxyde d'indium et oxyde d'étain est de 6 : 1 à 1 : 6, sur la base d'un rapport de poids, dans lequel le diamètre moyen est compris dans la plage de 50 à 150 nm, et la longueur est comprise entre 100 nm et 10 µm.
